

June 22, 1926.

1,590,113

J. F. MURPHY

METHOD OF TREATING HATS

Filed Sept. 14, 1925



Patented June 22, 1926.

1,590,113

# UNITED STATES PATENT OFFICE.

JAMES F. MURPHY, OF DANBURY, CONNECTICUT.

## METHOD OF TREATING HATS.

Application filed September 14, 1925. Serial No. 56,262.

This invention relates to a step in the method of making velour hats, and has for an object to so treat the fibres on and adjacent the surface of the hat that they will be 5 softened and loosened up during the brushing operation, so that they are pulled out in the desired manner by the brush and lie parallel for considerable length, and give an improved surface and a greater lustre to 10 the finished hat. This process softens the fibres on and adjacent the surface of the hat so that they are more easily disengaged from their union with one another by the brush, and thereby produce a longer fibre of 15 protrusion with far less waste of fur by broken fibres.

It is also an object of the invention to produce a method of treating hats which will give this improved surface and finish in 20 a much less time, so that with my method I am not only enabled to secure a much improved finish over the methods now generally employed, but I can finish the hats in a much shorter time, thus greatly reducing 25 the cost of manufacture.

With the foregoing and other objects in view, I have devised devices for carrying out my improved method which are illustrated in the accompanying drawing, similar 30 reference characters being employed throughout the various figures to indicate corresponding elements. In this drawing,

Fig. 1 is a front elevation of one form of device for treating hats by my improved 35 method.

Fig. 2 is a detail section showing the means of feeding steam to the interior of the hat supporting block.

Fig. 2<sup>A</sup> is a top plan view of one of the 40 steam funnels shown in Fig. 1.

Fig. 3 is a front elevation of another form of device for my improved method.

Fig. 4 is a transverse section thereof substantially on line 4-4 of Fig. 3.

Fig. 5 is a view similar to Fig. 3 showing a slightly different construction of device, and

Fig. 6 is an end elevation of the device shown in Fig. 5, certain parts being broken 50 away to more clearly show the construction.

My improved method of treating hats consists primarily in applying to the fibres of the hat, especially those on and adjacent the surface to be treated, a small amount of steam which softens and loosens the fibres, and brushing the hat while these fibres are

still softened and loosened by the action of the steam. To secure this effect the steam is applied either at the same time the hat is being brushed, or immediately before brushing, so that the fibre is brushed before the effect of the steam thereon has disappeared. The effect of the steam on the fibres disappears very rapidly, and therefore, if the steam is not applied during 60 the brushing operation it should be applied immediately before the brushing operation so that the brushing is practically coincident therewith.

In the devices shown on the drawing, that 70 shown in Fig. 1 is for use where the brushing operation is done by hand with a hand brush, and in this device the steam may be applied to the hat externally immediately before the brushing operation or internally 75 during the brushing operation or both. For this purpose a suitable stand 10 carries a rotatable shaft 11 driven from any suitable source of power, such as the crossed belt 12 and the straight belt 13 leading from any 80 suitable countershaft, not shown, to the idling pulleys 14 and 15 respectively on the shaft 11, and the usual means, not shown, for shifting these belts alternately to the fixed pulley 16 for reversing the direction 85 of rotation of the shaft.

At the outer end of the shaft is the block 17 for carrying the hat 18 to be treated, this block being of such a size that the crown of the hat fits snugly over the block and is 90 held thereby, the block forming a backing to support the hat during the brushing operation and, of course, the hat rotates with the block. Below the block is a steam funnel 19 with a flared upper end which is 95 preferably oblong in shape, and the open end is preferably covered with a piece of burlap 20 so that as the steam comes through the burlap it is equally distributed over the surface of the hat. Steam is supplied 100 to the funnel from a suitable source of supply, not shown, through the pipe 21, and a valve 22 in this pipe is controlled by a foot treadle 23.

Means is also provided for feeding steam 105 to the hat through the hat supporting block. For this purpose the shaft 11 is made hollow with a longitudinally extending passage 40, and it is internally threaded at its outer end to receive the externally threaded 110 nipple 41 of the block 17 whereby this block is secured to the shaft. The nip-

ple 41 is also internally threaded to receive the bushing 42 which has a bearing on the steam pipe 43, the pipe being turned down to give a running bearing in this bushing. The block 17 is provided with suitable small openings 46 to distribute the steam to the hat. The pipe 43 projects outwardly from the opposite end of the shaft where it is connected by means of the pipe 44 with the steam supply pipe 21 through a control valve 45. The valve 45 is operated by a treadle 47. It is preferred to mount two of these shafts 11 in the frame 10 and in reversed relation, as shown in Fig. 1.

In the operation of this device the hat to be treated is slipped over the block by which it is rotated, and by pressing on the treadle 31 a small amount of steam may be admitted to the funnel 19 which passes through the burlap and rises about the rotating hat. The moisture and heat of the steam softens and loosens the fibres at and adjacent the surface of the hat which is immediately brushed by the operator by holding the wire brush against the surface of the hat as it rotates, the supply of steam being cut off immediately prior to the brushing operation for the protection of the operator, but as no handling of the hat is required between the application of the steam and the brushing operation the brushing is done practically coincident with the application of the steam, so that the brushing is done while the fibres are still softened and loosened by the steam. Thus with this arrangement although the effect of the steam on the fibres is very quickly dissipated the brushing may be done while the fibres are still under the influence of the steam. If it is preferred to apply the steam to the hat during or coincident with the brushing operation this may be done by pressing on the treadle 47. This will admit steam to the block 17 through the pipe 44, and this steam will issue to the hat through the openings 46. It will also be apparent that steam may be applied both to the interior and exterior of the hat at the same time. During the treatment of the hat it must be brushed in opposite directions. Therefore, after the hat has been treated with the steam and brushed, by shifting the belts it may be rotated in the opposite direction, again treated with the steam and brushed while rotating in this direction, and so on, that is, treated and brushed while rotating in opposite directions as often as is found desirable. By placing blocks 17 at opposite ends of the shafts, as shown, two hats may be treated by different operators at the same time, or, if it is desired not to reverse direction of rotation of the shafts, the hat may be treated while rotating in one direction on one of the blocks and then transferred to the other block, which, as it is reversed, will have the effect of

rotating the hat in the opposite direction so that it may be treated accordingly.

In Figs. 3 to 6 I have shown a device for carrying out my method in which the brush is driven by power means. In this construction the circular wire brushes 24 are mounted on a rotatable shaft 25 carried by a frame or stand 10 and operated by the belts 12 and 13 in the same manner as the hat supporting blocks in the first form. Mounted adjacent the periphery of the brush and extending transversely thereof is a tubular support 26 for the hat 27. This support is provided with lateral openings 28, preferably directed toward the brush, the free ends of the support being closed, and the support is connected by means of a pipe 29 to any suitable source of steam not shown. The supply of steam to this support is controlled by a valve 30 through a treadle 31. It is to be noted that there are two brushes mounted on the shaft at the opposite sides of the stand, and that the supports 26 are arranged in reversed relation so that the free end thereof is arranged at the left side of the right hand brush, and the free end of the other support is arranged at the right hand side of the left hand brush, as viewed in Fig. 3. In operation the hat 27 is slipped between the support and brush as shown in Fig. 4, the support holding the surface of the hat against the surface of the brush. As the brush rotates it rotates the hat on the support, the speed of rotation of the hat being controlled more or less by the operator as he holds the hat on the support. As the hat is being brushed the fibres are softened and loosened by the application of a small amount of steam through the openings 28. In this form the steam may be applied during the brushing operation, and by sliding the hat in or out on the support practically the entire outer surface may be brushed. The rotation of the brushes may be reversed to give the brushing effect in opposite directions, or the brushes may be rotated continuously in the same direction and after it is brushed on the right hand brush it may be brushed in the opposite direction by transferring it to the left hand brush, and as the support for this brush is reversed from that of the first brush it will be obvious the hat will be brushed in the opposite direction. It is preferred to enclose the brushes in a hood 32 and connect this hood with an exhaust fan 33 so as to remove the fibres which are torn from the hat during the brushing operation, this fan discharging into a suitable collecting box or bag not shown, for salvaging the fur or fibre removed.

In Figs. 5 and 6 is shown a device which operates substantially the same as that shown in Figs. 3 and 4, except that it is used mostly for brushing the brims of the

hats. In this form the hat support comprises a small hollow block 34 having a curved surface toward the brush which is provided with discharge openings 35. Steam is supplied to this port through a pipe 36 controlled by the valve 37, the same as in the other form, and the pipe 36 is connected to the back of the support. By this arrangement the brim of the hat may be brushed in opposite directions without reversing the brush by simply inserting the brim from one side of the support and brushing it and then removing it and inserting it from the other side of the support, which will brush it in the opposite direction. In this form, as in the forms shown in Figs. 1, 3 and 4, the steam may be applied during the brushing operation. I have found that although brushes having steel wires extending radially of the brush give a satisfactory result, still I prefer that the wires 38 should be bent intermediate their ends so that the outer portion 39 will be inclined in the direction of rotation of the brush as shown in Figs. 4 and 6. Thus the wires at the time of engaging the hat surface, instead of being normal to the surface, are inclined thereto at an acute angle, and I have found that with this arrangement the wires pass more readily through the fibres and lay them out properly with a less tearing and breaking of the fibres than when they are normal to the surface of the hat. With my improved method not only do I secure a much improved surface and finish on the hat, but I can secure this finish much more rapidly or in less time so that it is obtained at much less cost. The application of a small amount of steam to the fibres of the hat during the brushing operation, or such a short time before the brushing operation that the fibres are still under the influence of the steam, softens and loosens the fibres so that they will more easily disengage from their union with one another

under the action of the brush. The brush, therefore, passes more easily through and between the fibres laying them out in the required parallel relation to give a longer fibre of protrusion with far less waste of fur by tearing or breaking of the fibres by the brush than where they are brushed dry. When the hat surface is brushed dry it is merely the surface fibres which are brushed up, and the brush does not get into the fibres and pull them up to give the required length of free fibre as it does when the steam is applied, as in the above described method. The heat and moisture of the steam softens and loosens up the fibres so that one end is pulled out by the brush and they lie parallel for some length. They are then blown up by a suitable air blast and clipped to the proper length by clippers. It has been found in practice that this treatment gives a very beautiful soft finish which has much more lustre than is secured where the hats are brushed dry.

Having thus set forth the nature of my invention what I claim is:

1. The step in the method of making a velour hat which consists in raising the nap by treating the hat body with sufficient steam to soften and loosen the fibres adjacent the surface of the hat, and brushing the surface of the hat while the fibres are under the influence of the steam to loosen and draw out free one end of the fibres.

2. The step in the method of making a velour hat which consists in raising the nap by treating the hat body with sufficient steam to soften and loosen the fibres adjacent the surface of the hat, and brushing the surface of the hat simultaneously with the application of the steam to loosen and draw out free one end of the fibres.

In testimony whereof I affix my signature.

JAMES F. MURPHY.